

## UNITED STATES PATENT OFFICE

MILTON O. SCHUR, ROYAL H. RASCH, AND BENJAMIN G. HOOS, OF BERLIN, NEW HAMPSHIRE, ASSIGNEES TO BROWN COMPANY, OF BERLIN, NEW HAMPSHIRE, A CORPORATION OF MAINE

## CONDITIONING OF CELLULOSE FIBER AND THE PRODUCT THEREOF

No Drawing.

Application filed December 14, 1928. Serial No. 326,150.

This invention relates to conditioning, prior to nitration, of cellulose fiber to produce a product useful for the manufacture of films, lacquers, artificial silk, and the like.

5 Before cellulose fiber is subjected to nitration, it has sometimes been found desirable to condition the fiber so as to make possible high yield and good quality of nitrated product. For instance, in application Serial No.

10 140,674, filed October 9, 1926, by George A. Richter, Milton O. Schur, and Royal H.

Rasch, there are disclosed various methods of treating the fiber so as to retard the action of the nitrating acid, as it has been found that improved results are thereby realized.

15 Nitration may be retarded, as by beating the fiber, treating it with nitrocellulose, or otherwise suitably lowering its absorptivity, as by sheeting into tissue paper and subjecting 20 to heavy pressure before drying. The theory advanced in that application is that the sulphuric acid in the nitrating bath tends to hydrolyze the cellulose fibers, especially when the pulp is highly absorptive. If, however, the fiber is first treated with nitrocellulose or is otherwise rendered less absorptive, the side reaction is apparently retarded or avoided and nitration proceeds smoothly.

25 The coating or film of nitrocellulose on the fibers probably permits nitric acid to penetrate into the fiber wall more easily than sulphuric acid, and perhaps readily allows water generated within the fiber during nitration to diffuse into the main body of the

30 nitrating acid, so that within the fiber wall there is believed to be a nitric-acid-rich mixture which has a greatly reduced hydrolyzing effect and nitrates the cellulose before hydrolysis can proceed to any troublesome degree.

35 It is well known, for example, that nitrating acids rich in nitric acid give high yields, but that acids rich in sulphuric acid cause hydrolysis and correspondingly low yields. The film of nitrocellulose on the

40 fibers, by slowing up the reaction, eliminates local over-heating in the acid bath, and thus prevents loss in yield, for the higher the temperature of nitration, the greater is the tendency for the yield to drop because of side reaction. When using fiber in the form of tis-

sue, another function of the nitrocellulose is to cement the loosely adhering surface fibers to the body of the paper, thereby counteracting the tendency of the nitrated surface fibers to pass into solution in the nitrating acid and become lost during the separation of the spent acid from the nitrocellulose in the centrifuge.

45 We have discovered that if cellulose fiber is treated with an organic solvent of substances such as the resins or waxes naturally occurring therein, and then evaporated from the fiber, the yield of nitrated product is notably increased and when the product is dissolved in suitable media, solutions of remarkable clarity and sparkle are produced. Upon making this discovery, we at first found it difficult to account for the surprising results secured, but study and research indicate a consistency between these results and the theory which we have advanced. 50 Our conclusion is that a solvent of the character described, when evaporated from cellulose fibers, deposits on the surface of the fibers a film of the resinous or waxy materials naturally occurring therein, and that the film acts in a manner similar to a nitrocellulose film deposited on the fiber before nitration as heretofore described. We were led to this conclusion through the observation that the fibers after treatment with such solvents absorb water less readily than previously, that solvents of widely different characteristics produce similar results, that the initial temperature rise in the nitrating 55 bath is 0.1° to 0.3° C. less than with untreated fiber, and finally that the results are so strikingly similar to those obtained when the fiber is treated with nitrocellulose before nitration.

60 In carrying out a treatment of the fiber with solvent, the conditions maintained may be such that little, if any, extraction of resinous or waxy materials from the fiber is effected. Thus, we have found that the mere moistening or wetting of fluffy or finely shredded wood pulp or tissue with solvent, followed by the evaporation of the solvent, results in an increase in yield of nitrated product, and that improved results are se- 65 70 75 80 85 90 95 100

cured even when the fiber is subjected to the action of vapors of the solvent. The treatment may be carried out with a great variety of organic solvents, it being advantageous to use non-inflammable solvents, such as carbon tetrachloride, particularly when the fiber is subjected to vapors of the solvent, thus avoiding explosion and fire hazard. When the fiber is one having comparatively high resin content, such as sulphite pulp, the solvent treatment may be carried out so as to effect an extraction and removal of a portion of the resin, sufficient resin being left so that when the solvent is evaporated, an acid-repellent film which retards nitration of the fiber is left on its surface. The fiber may be immersed in bulk form in the solvent or passed through a bath of solvent as a continuous sheet of tissue, under conditions resulting in an extraction of resinous, waxy, and oily impurities from the fiber, so that nitrocellulose or high stability and freedom from coloring matter may be prepared therefrom. While such impurities may be substantially completely removed from the fiber, there is a trace of resinous and waxy material left after any practical treatment, this trace apparently being deposited on the surface of the fiber when the solvent is evaporated. This trace is ordinarily negligible with regard to imparting color, cloudiness, instability, etc., to the nitrocellulose prepared from the fiber, and from this viewpoint the fiber may be properly described as having been substantially completely free from resinous and waxy material. From the viewpoint of yield, however, the presence of this minute residue on the surface of the fiber is of high advantage. In the case of wood pulp which has been refined to high alpha cellulose content, as by boiling in an alkaline liquor containing soap, non-alpha cellulose impurities, including beta and gamma celluloses, lignin, resinous, waxy, and oily substance, are largely removed from the fiber. But traces of resinous and waxy material are left in the fiber because of practical limitations in a refining process, and since only traces are needed to form an acid-repelling film on the fibers, it becomes possible, through the expedient of treating the fiber with a solvent, to put the residual waxy material to advantageous use. For instance, when a tissue of the refined wood fiber is dipped in solvent, the solvent evaporated, and the tissue nitrated, it is found that a noteworthy increase in yield of nitrocellulose is effected. Inasmuch as the refined fiber contains only traces of waxy or resinous material, very little extraction of such material is effected when a tissue of such fiber is dipped in solvent for a short time. The treatment with solvent may be effected under various temperature conditions, the sol-

vent being from room temperature to its boiling point, or in the form of a vapor.

Below is a table showing the yield of nitrocellulose obtained after sheets of waterleaf tissue made of a wood pulp of high alpha cellulose content were dipped for a second or two in various solvents at room temperature, dried, and bone-dried at 100° to 103° C. prior to nitration:

|                  |             |    |
|------------------|-------------|----|
| Iso-amyl alcohol | 154.2       | 75 |
| Iso-amyl acetate | 154.3       |    |
| Ether            | 153.3       |    |
| Alcohol (98%)    | 154.0       |    |
| Chloroform       | 153.7       | 80 |
| Trichlorethylene | 154.0       |    |
| Gasoline         | 154.8       |    |
| Kerosene         | 154.2       |    |
| Benzol           | 154.2       |    |
| Benzol-acetone   | 155.5-152.5 | 85 |

(The yield obtained by nitrating similar sheets of tissue which were untreated with solvent was from 146 to 151.)

It is thus seen that a great variety of organic solvents may be employed for the purpose desired. Inasmuch as the solvents may be substantially completely removed from the fiber prior to nitration, no impurities which affect the purity or stability of the product are introduced into the fiber. 95

Various modifications are possible in practising the process of the present invention. Thus, mixtures of solvents may sometimes be used to better advantage than one solvent alone. For instance, although acetone by itself raises the yield very little, it may be used as a comparatively inexpensive vehicle to carry the much more effective but more expensive iso-amyl acetate through a paper sheet. Beneficial effects may also be obtained by passing a sheet of dry paper through a chamber containing air heavily charged with vapors of the solvents. 105

While the process of the present invention may be employed in preparing cellulose fibers of various origins for nitration, it may be applied to especial advantage in the case of wood pulp, as such fiber may be improved more markedly as a raw material for nitration than cotton fiber. We have in mind more particularly a wood pulp which has been refined to high alpha cellulose content, as such pulp yields nitrocelluloses comparable in quality with those prepared from cotton fiber. Such pulp, however, may fail under some circumstances to give as high a yield of nitrocelluloses as cotton fiber, but by treating such refined wood pulp with solvents as herein described, it is possible to raise the yield of nitrocellulose to a substantially theoretically perfect value. 115

Having thus described certain modes of practising the process of this invention, it should be evident to those skilled in the art that various changes and modifications might 130

be made therein without departing from the spirit or scope of invention as defined by the appended claims.

We claim:

5. 1. A process which comprises treating cellulose fiber with an organic solvent of a substance naturally occurring therein, evaporating the solvent from the whole surface of the fiber, and nitrating the fiber.
10. 2. A process which comprises wetting cellulose fiber with an organic solvent of a substance naturally occurring therein, evaporating the solvent from the whole surface of the fiber, and nitrating the fiber.
15. 3. A process which comprises wetting cellulose fiber with a non-inflammable organic solvent, evaporating the solvent from the whole surface of the fiber, and nitrating the fiber.
20. 4. A process which comprises dipping a tissue of cellulose fiber into an organic solvent of a substance naturally occurring therein, evaporating the solvent from the whole surface of the tissue, and nitrating the tissue.
25. 5. A process which comprises wetting wood pulp with an organic solvent of the resinous and waxy materials naturally occurring therein, evaporating the solvent from the whole surface of the fiber, and nitrating the pulp.
30. 6. A process which comprises immersing a tissue of wood pulp in a bath of an organic solvent of the resinous and waxy materials naturally occurring in such pulp, evaporating the solvent from the whole surface of the tissue, and nitrating.
35. 7. A dry, waterleaf paper which has undergone previous treatment with an organic solvent of residual resinous and waxy material associated with the cellulose fibers constituting such paper and then dried to evaporate said solvent from the whole surface of said paper, whereby said surface is enriched with resinous and waxy material.
40. 8. A dry, waterleaf paper composed of wood pulp and which has undergone previous treatment with an organic solvent of residual resinous and waxy material associated with the pulp fibers and then dried to evaporate said solvent from the whole surface of said paper, whereby said surface is enriched with resinous and waxy material.
45. 9. A dry, waterleaf paper composed of wood pulp of high alpha cellulose content and which has undergone previous treatment with an organic solvent of residual resinous and waxy material associated with the pulp fibers and then dried to evaporate said solvent from the whole surface of said paper, whereby said surface is enriched with resinous and waxy material.
50. 10. A process which comprises treating cellulose fiber with an organic solvent of a substance naturally occurring therein while substantially keeping said substance in said
- fiber, evaporating the solvent from the whole surface of the fiber, and nitrating the fiber.
11. A process which comprises treating refined wood pulp with an organic solvent of the resinous and waxy substances naturally occurring therein while substantially keeping said substances in said pulp, evaporating the solvent from the whole surface of the fiber, and nitrating the pulp.
12. Cellulose fiber wherein resinous and waxy constituents have merely undergone migration to its surface through treatment with a solvent for said constituents, and drying its entire surface while keeping said constituents in said fiber.
13. Refined wood pulp wherein residual resinous and waxy constituents have merely undergone migration to its surface through treatment with a solvent for said constituents, and drying its entire surface while keeping said constituents in said pulp.
14. A tissue of cellulose fiber wherein resinous and waxy constituents have merely undergone migration to its surface through treatment of said tissue with a solvent for said constituents, and drying its entire surface while keeping said constituents in said tissue.
15. A tissue of refined wood pulp wherein residual resinous and waxy constituents have merely undergone migration to its surface through treatment of said tissue with a solvent for said constituents, and drying its entire surface while keeping said constituents in said tissue.
- In testimony whereof we have affixed our signatures.
- MILTON O. SCHUR.  
ROYAL H. RASCH.  
BENJAMIN G. HOOS.